

## UNITED STATES PATENT OFFICE

2,234,047

## HIGH CREEP STRENGTH LOW ALLOY STEEL

Harry L. Frevert, Philadelphia, Pa., assignor to  
The Midvale Company, Philadelphia, Pa., a corporation of DelawareNo Drawing. Application November 14, 1939,  
Serial No. 304,329

4 Claims. (Cl. 75—126)

There are certain articles of manufacture, now made of steel, alloyed or not with one or more of the common steel-alloying elements, and which in use are subjected to high temperatures, commonly within the range of 800—1100° F., which it is highly desirable should have the qualities of high "creep strength" and freedom from brittleness. "Creep strength" may be roughly defined as that quality enabling the article to resist continuous deformation under constant load at high temperature. It is also essential that these qualities should be maintained for a long period of time. It is well recognized that these articles subjected to such high temperatures, and particularly those which normally must function at such high temperatures continuously for prolonged periods of time, do not exhibit these qualities to a satisfactory degree, unless made of expensive, highly alloyed compositions.

20 The development of an inexpensive forging steel that will resist "creep" at temperatures practically up to incandescence is the object of my invention. The problem presents unusual difficulties in view of the long time required experimentally to determine whether or not given compositions are durable with respect to the qualities sought, since the behavior of different compositions, found on long time tests to retain the desired qualities for markedly different periods of time, do not, on short time tests, exhibit any variance sufficient to predicate therefrom the length of time during which such qualities may be expected to be maintained.

25 In the manufacture of many such articles the use of straight low carbon steel has been found to be open to fewer objections than most of the commercial alloy steels. Commercial alloy steels generally contain one or more of the common alloying elements in considerable proportions, such proportions being often of value and importance in securing other qualities than those above mentioned.

30 In view of the lack of superiority of commercial alloy steels over low carbon steel, in my investigation of the problem it occurred to me to determine the effect of the addition of very small amounts of different alloying elements. The result of my experimental work, which has necessarily continued over a long period of time, is the discovery that the addition of certain elements, provided each is added in certain very small proportions, does substantially increase creep strength without impairment of, and indeed with improvement in, other qualities essential or desirable in those articles of manufacture for which the alloy steel is primarily intended. It was found, also, with respect to certain of these elements, that increasing the amount added beyond a certain quite low percentage not only failed to give better creep strength but acted in a direction

the reverse to that exhibited by their addition in lower percentage. With respect to certain other elements it was found that increase of the amount added beyond a limited range does not improve the steel in respect to this quality, or does not improve it to any material extent, and that such increase is open to objections of so serious a nature as not to warrant the use of the elements beyond the low percentage which approaches the optimum for the attainment of the best results.

5 The elements that have been found to give cheaply the results sought, when all are added and when each is added in a certain small proportion, are manganese, silicon, chromium and molybdenum. The addition of increased proportions of these elements has been found to be not only ineffective, but even to impair the qualities produced by the addition of these elements in the amounts specified.

10 Metallurgists are of course quite familiar with 20 alloy steels containing the particular combination of elements above specified, but the art is devoid of any discovery that this particular combination of elements, each added in very small percentage within a particular narrow range, is essential to 25 secure the particular qualities mentioned in the forepart of this specification without sacrifice of other necessary qualities.

15 Considering in order the alloys specified, manganese is added in an amount which is not uncommon, namely between .50 and 1.25%. Its addition somewhat beyond the maximum specified does not decrease creep strength, but a larger amount makes the metal more difficult to forge 30 in large sizes and more sensitive to hardening under normal cooling conditions and causes the highly objectionable condition known in the art as "banded ferrite." It is desirable not to add more 35 than about one per cent.

20 The addition of silicon is of some importance 40 but preferably it should not be present in a proportion above 4%. With a percentage of silicon beyond 4%, the creep resistance decreases at an accelerating rate.

25 The optimum proportion of chromium is about 45 .6%, but within the range of .5 to 1% its effect in increasing creep resistance is pronounced. Increasing the percentage of chromium beyond the maximum specified has the opposite effect.

30 The addition of as little as .15% molybdenum 50 has a substantial effect in increasing creep resistance. As the amount of molybdenum increases, the creep resistance also increases, although at a progressively decreasing rate. If molybdenum be added beyond .75% there is no 55 increase of creep resistance commensurate with the added cost and the steel becomes more difficult to work.

35 The total of the specified four added alloying elements should not therefore exceed 3.4% and 60

optimum conditions are satisfied by the addition of about 2%; a steel containing Mn 1.0%, Si .2%, Cr .6% and Mo .2% being not far from an ideal composition.

5 The carbon is preferably quite low, say not over about .25%, although it is permissible to have any carbon content not over about .5%.

It should be noted that the composition approaches more nearly that of carbon steel than 10 do most alloy steels, although its improvement over carbon steel is striking.

As indicating the pronounced effect of adding 15 chromium and molybdenum to carbon steel containing manganese and silicon within the ranges above specified, the following comparison of the 15 creep values of different compositions were obtained:

| 20 | C       | Mn   | Si  | Cr  | Mo  | Load producing 1%/100,000-hrs. creep rate |         |          |          |
|----|---------|------|-----|-----|-----|-------------------------------------------|---------|----------|----------|
|    |         |      |     |     |     | 800° F.                                   | 900° F. | 1000° F. | 1100° F. |
| 25 | (a) .26 | .65  | .35 | —   | —   | 11,800                                    | 6,600   | 3,000    | 1,820    |
|    | (b) .24 | 1.05 | .26 | —   | —   | 12,000                                    | 4,300   | —        | —        |
|    | (c) .24 | 1.25 | .18 | —   | —   | 25,200                                    | 14,000  | —        | —        |
|    | (d) .25 | .95  | .20 | .62 | 20  | 44,500                                    | 25,500  | 9,000    | —        |
|    | (e) .26 | .50  | .19 | .43 | .15 | 20,000                                    | 12,600  | 6,400    | 3,000    |

30 The results obtained on experimental composition (d) were confirmed by a three-ton heat in which the composition (f)—C .26, Mn .88, Si .17, Cr .60 and Mo .20—was nearly identical with composition (d).

35 Composition (a) does not meet requirements. Nor does composition (b), even though the percentage of manganese is increased to about what has been found to be the probably most effective proportion in the complete composition. When, 40 however, the percentage of manganese is increased to about the maximum, and a very small proportion of molybdenum is added, a pronounced improvement results, as is illustrated by composition (c). When to this composition is 45 added a very small percentage of chromium as in composition (d), then the improvement is quite remarkable. However, as shown in composition (e), a reduction in manganese, chromium and molybdenum produces a composition inferior to 50 composition (c) which contains no chromium. This indicates that nearly twice the percentage of molybdenum will not compensate for low manganese and low chromium.

55 It was also found, in outside tests, by prospective users of compositions essentially the same as (d) and (f), that after loading at 1022° F. for 2200 hrs. the metal or composition has not undergone any deterioration, its elastic limit, ductility and Charpy impact values having as a matter of 60 fact increased. Tests before and after loading at 1022° F. for 2200 hrs. follow:

| 65 |                            | T. S.   | E. L.  | Elong. | Red. | Charpy, ft. lbs. |
|----|----------------------------|---------|--------|--------|------|------------------|
|    | Before testing at 1022° F. | 108,700 | 44,000 | 21.0   | 53.8 | 18.8             |
|    | After testing at 1022° F.  | 108,000 | 59,000 | 25.0   | 58.6 | 28.3             |
|    |                            | 95,800  | 59,000 | 25.7   | 59.7 | 27.0             |

70 These data show that this material not only has a creep value of the order of practically four times that of carbon steel but that unlike many steels otherwise useful for high temperature service it does not undergo embrittlement.

75 Tests to determine the load required to frac-

ture this material over long periods of time produced the following results:

| Temperature, °F. | Load to produce rupture in 100,000 hrs. P. S. I. | 5  |
|------------------|--------------------------------------------------|----|
| 900              | 39,000                                           |    |
| 1000             | 21,500                                           |    |
| 1100             | 5,500                                            | 10 |

Fractures produced in rupturing bars incident to determining, by extrapolation, the above figures all showed ductile transcrystalline fractures as opposed to the brittle, intercrystalline fracture of steels which fail suddenly and without warning at such temperatures. These tests were made on material simply air quenched from 1550° F. and drawn at 1200° F., which treatment confers a fine microstructure without free ferrite. 15

The only element not specified that I have 20 discovered to have a beneficial effect in attaining the object of the invention is tungsten, which is much more expensive than molybdenum and to produce the same effect as molybdenum must be added in much larger proportion. In specifying, 25 in the claims, after enumerating the elements above described, that the balance of the composition is substantially iron, it is not intended to exclude the addition of an inconsiderable amount of any other element that is ineffective to materially reduce the efficiency of the elements specified. 30

It will be noted that the total percentages of 35 alloying elements other than the carbon in compositions (d) and (f) are respectively 1.97 and 1.85%. The total percentage of these four elements should not exceed about 3.4% or be less than 1.25% and preferably should be between 1.5 and 2.5%. In all cases the percentage of either manganese or chromium should not be much 40 less than, and should usually exceed, that of the molybdenum; and the percentage of silicon should generally be less than that of any of the other elements except carbon, and always less than that of the manganese or the chromium. 45

For many purposes the composition has slight 50 advantage over carbon steel of equivalent strength, but for many other uses, the creep resistance, the maintenance of that resistance with prolonged use, and freedom from cold embrittlement after prolonged high temperature exposure, 55 that characterize my improved composition, are of the utmost importance and value. Among articles of manufacture for such use may be mentioned ovens, autoclaves, and other reaction chambers and vessels, turbine spindles and other turbine elements (wherein very slight "creep" is a serious matter), heat exchangers, tubing and piping, bolts and nuts.

What I claim and desire to protect by Letters 60 Patent is:

1. An alloy having a high and durable creep 65 strength and freedom from cold embrittlement after prolonged high temperature exposure containing carbon not over .5% and the addition elements manganese, silicon, chromium and molybdenum, the manganese being present in a proportion between .65 and 1.5%, the chromium in a proportion between .5 and 1.0%, the silicon in a proportion between .15 and .40%, and the molybdenum in a proportion between .15 and .50% and having the further characteristic that the percentage of manganese is not less than the percentage of chromium plus the percentage of molybdenum and that the percentage of chro- 70 75

mium is in excess of the percentage of molybdenum and in excess of the percentage of silicon, the balance of the composition being substantially all iron.

5. 2. An alloy having a high and durable creep strength and freedom from cold embrittlement after prolonged high temperature exposure containing carbon not over .5% and the addition elements manganese, silicon, chromium and molybdenum, the manganese being present in a proportion between .65 and 1.5%, the chromium in a proportion between .5 and .9%, the silicon in a proportion between .15 and .40%, and the molybdenum in a proportion between .10 and .50% and having the further characteristic that the percentage of manganese is not less than the percentage of chromium plus the percentage of either of the remaining two addition elements and that the percentage of chromium is in excess of the percentage of molybdenum and in excess of the percentage of silicon, the balance of the composition being substantially all iron.
15. 3. An alloy having a high and durable creep strength and freedom from cold embrittlement after prolonged high temperature exposure containing carbon not over .5% and the addition elements manganese, silicon, chromium and molybdenum, the manganese being present in a

proportion between .85 and 1.1%, the chromium in a proportion between .5 and .9%, the silicon in a proportion between .15 and .3% and the molybdenum in a proportion between .15 and .4% and being further characterized by the fact 5 that the percentage of manganese is not substantially less than the percentage of chromium plus the percentage of the remaining two addition elements and that the percentage of chromium is not substantially less than approximately 10 the percentage of silicon and molybdenum combined, the balance of the composition being substantially all iron.

20. 4. An alloy steel having a high and durable creep strength and freedom from cold embrittlement after prolonged high temperature exposure containing carbon less than .50% and the additional elements manganese, silicon, chromium and molybdenum in a total percentage between 1.5 and 3.4 per cent., the relative proportions of 15 the addition elements being so adjusted that the percentage of manganese is not less than the percentage of chromium plus the percentage of molybdenum and that the percentage of chromium substantially exceeds the percentage of 20 either molybdenum or silicon, the balance of the composition being substantially all iron.

HARRY L. FREVERT.